

J. W. BRAINARD,  
MANUFACTURE OF HOOPS,  
APPLICATION FILED DEC. 29, 1914.

1,273,139.

Patented July 23, 1918

FIG. 1



FIG. 2



FIG. 4



FIG. 3



FIG. 5



WITNESSES

*W. T. Johnson*  
*R. D. Little*

INVENTOR

*J. W. Brainard*  
*J. C. Leuthenzer*  
*his Attorney*

# UNITED STATES PATENT OFFICE.

JAMES W. BRAINARD, OF PITTSBURGH, PENNSYLVANIA.

## MANUFACTURE OF HOOPS.

1,273,139.

Specification of Letters Patent. Patented July 23, 1918.

Application filed December 29, 1914. Serial No. 879,479.

To all whom it may concern:

Be it known that I, JAMES W. BRAINARD, a citizen of the United States, and resident of Pittsburgh, in the county of Allegheny and State of Pennsylvania, have invented certain new and useful Improvements in the Manufacture of Hoops, of which the following is a specification.

My invention relates to the manufacture of metal hoops for barrels and kegs, and while not restricted to such uses more particularly relates to the manufacture of beaded chime hoops used on slack cooperage.

Flat metal hoops have been extensively used within recent years as a substitute for hoops formed of wood. It has been found that the metal hoops will stretch or elongate after being applied to the barrels and kegs, the hoops stretching to such an extent as to become loosened and fall off the ends of the barrels or kegs in the severe usage which the packages must resist in the frequent handling operations to which the packages are necessarily subjected in storing and transportation.

My invention is designed primarily to overcome these difficulties and to provide a hoop having superior physical qualities, which will not stretch after being placed in position on the chime or bilge of a barrel or keg.

Another object of my invention is to provide a hoop having a surface which is particularly adapted for painting or galvanizing.

Still further objects of my invention will become apparent as the invention is more fully described hereinafter and is specifically pointed out in the appended claims.

Referring now to the accompanying drawings, Figure 1 is a longitudinal section of a portion of a barrel showing one form of chime and of bilge hoop, made and applied for use on the barrel, in accordance with my invention.

Fig. 2 is a detail sectional elevation of the chime hoop shown in Fig. 1.

Fig. 3 is a transverse section, showing the bilge hoop of Fig. 1.

Figs. 4 and 5, are similar transverse sections showing modified forms of beaded chime hoops.

In the drawings forming part of this specification, the numeral 2 designates a barrel or keg having a chime hoop 3 and bilge hoop 4. The chime hoop 3 is provided with a

hollow bead 5 on one edge which is formed as is shown in detail in Fig. 2, and the bilge hoop 4 has a middle corrugation 6 and at its lower edge an outwardly and downwardly inclined lip 7, as shown in detail in Fig. 3.

In Fig. 4 the chime hoop 3<sup>a</sup> has a bead 5<sup>a</sup> which is curled or curved to a greater extent than the hoop of Fig. 2, and in Fig. 5 the bead 5<sup>b</sup> on the hoop 3<sup>b</sup> is flattened.

In carrying out my invention the hoop metal is rolled in a hot mill to within three or four gages of the particular thickness or gage of material desired in making the particular size of hoop required. The hoop metal is then cold rolled so as to reduce the gage or thickness of the hoop metal to that desired.

The hoop metal after being cold rolled is then cut into pieces of the required length, and the pieces are beaded on one or both edges in the manner shown in the drawings, and punched. The ends of the hoops are then riveted or otherwise fastened together and the hoop is then flared to the desired taper.

In some cases the hoops are then galvanized after being pickled. In other cases the hoops will be painted and in the majority of cases no protective coating will be applied to the hoops.

Hoops of nine inches diameter ordinarily are made of hoop metal one and one eighth inches in width by about No. 24 B. W. gage.

Larger sizes are made of hoop metal up to two inches wide by No. 21 gage, the strips from which such hoops are made being as much as or even more than 13 feet long.

In the cold rolling operation, hoop metal of one and one eighth inches width by No. 19 or 20 B. W. gage is cold rolled to one and one eighth inches by No. 24 gage, and in this cold rolling operation the metal is stretched and densified (*i. e.* is permanently elongated and thereby stretched beyond the elastic limit of the metal) so that when later applied for use as a hoop to a barrel or keg, there will be no further stretching of the metal.

The cold rolling operation also removes the scale from the surfaces of the metal and in this way produces a surface requiring little or no pickling in preparation for galvanizing and an improved surface particularly well adapted for painting.

The cold rolling operation also increases the physical properties of the steel of which

the hoop is formed. Hoops made of hot finished material of one and one eighth inches width by No. 22 gage have an ultimate strength of approximately 60,400 pounds and the elongation in six inches is 1.12 per cent., while with the same material after being cold rolled to No. 24 gage the ultimate strength is 84,600 pounds and the percentage of elongation in six inches is reduced to .6 per cent.

Extended use of hoops made from metal cold rolled in this manner show that stretching of the hoops after being applied to the barrel, which ordinarily occurs when the barrel is handled, is entirely prevented and overcome, and a hoop of increased strength and durability is obtained.

The advantages of my invention will be apparent to those skilled in the art. By subjecting the material from which the hoops are made to a cold rolling operation, the stretch is taken out of the metal before beading and forming the hoops, so that when later applied to the barrels the hoops will not elongate or stretch while in service. In this way hoops are provided which will remain in place on the barrel and which will not become loosened when the key or barrel to which they are applied is frequently handled.

The manner of beading the hoops and the size of the hoops obviously may be varied and the beads may be omitted without de-

parting from my invention and other changes may be made within the scope of the appended claims. As the same result is obtained by cold drawing, the term cold rolled as used herein is intended to cover cold drawn as well as cold rolled materials.

I claim:

1. In the manufacture of metal hoops, the steps consisting in stretching hot rolled metal strips beyond the elastic limit of the metal by cold rolling, cutting the stretched metal to length and fastening one end of the cut lengths to the other to form the hoop.

2. In the manufacture of metal hoops, the steps consisting in stretching hot rolled metal strips beyond the elastic limit of the metal, cutting the stretched metal to length and fastening one end of the cut lengths to the other to form the hoop.

3. In the manufacture of metal hoops, the steps consisting in stretching hot rolled metal strips beyond the elastic limit of the metal, cutting the stretched metal to length and fastening one end of the cut length to the other, and then flaring the strips to form the hoop.

In testimony whereof, I have hereunto set my hand.

JAMES W. BRAINARD.

Witnesses:

R. N. McELHENY,  
JAMES W. HAMILTON.